

1

3,129,052

### NEW DYEING PROCESS

Timothy Leslie Dawson and Walter Percival Mills, Manchester, England, assignors to Imperial Chemical Industries Limited, London, England, a corporation of Great Britain

No Drawing. Filed Oct. 24, 1960, Ser. No. 64,285  
Claims priority, application Great Britain Nov. 13, 1959  
4 Claims. (Cl. 8—54)

This invention relates to a dyeing process and more particularly it relates to a process for dyeing natural and regenerated protein textile materials.

According to the invention there is provided a process for dyeing natural and regenerated protein textile materials with a water-soluble dyestuff which contains at least one group of the formula:  $-\text{X}-\text{CH}=\text{CH}_2$  wherein X represents a  $-\text{SO}_2-$  or



group and R represents a hydrogen atom or a substituted or unsubstituted hydrocarbon radical, which comprises dyeing the natural and regenerated protein textile material with an aqueous solution of the said dyestuff at a pH less than 7 and subsequently raising the pH during the dyeing process.

Each of the groups of the formula:  $-\text{X}-\text{CH}=\text{CH}_2$  is attached to a carbon atom present in the dyestuff molecule. The carbon atom may form part of an aryl ring present in the dyestuff molecule or may form part of an alkyl chain which is itself attached to an aryl ring. The dyestuff may be a member of the azo, which may be monoazo or polyazo, nitro, anthraquinone and phthalocyanine, which may be metal-containing phthalocyanine such as copper phthalocyanine, series which contains a water-solubilising group such as a sulphamyl or carboxylic acid group and preferably a sulphonate acid group. If desired the azo dyestuffs may contain coordinately bound metal such as coordinately bound copper, chromium or cobalt.

As examples of the substituted or unsubstituted hydrocarbon radicals represented by R there may be mentioned alkyl radicals for example lower alkyl radicals such as methyl, ethyl, propyl and butyl radicals which may contain substituents such as hydroxy, methoxy and ethoxy groups, aralkyl radicals for example benzyl and  $\beta$ -phenylethyl radicals, cycloalkyl radicals for example cyclohexyl radicals and aryl radicals for example monocyclic aryl radicals such as phenyl, tolyl and methoxyphenyl radicals. It is however preferred that R represents a hydrogen atom.

The process of the invention may be conveniently carried out by immersing the natural and regenerated protein textile material in an aqueous solution of the said dyestuff containing an acid or an acid salt so that the pH of the aqueous solution is less than 7 and is preferably between 2 and 7, heating the dyebath for a period at a suitable temperature, for example at a temperature between 80° C. and 100° C., adding an alkyl, an alkaline salt, or a salt which becomes alkaline when heated, to raise the pH of the dyebath, preferably to a pH of between 4.5 and 8, and heating for a further period at a suitable temperature, for example at a temperature be-

2

tween 80° C. and 100° C. The dyed textile material is then removed from the dyebath, rinsed in water and dried. If desired the dyed textile material may be given a soaping treatment, for example by heating the dyed textile material in an aqueous solution of soap or synthetic detergent, the aqueous solution optionally containing an alkali such as sodium carbonate.

As examples of the acids or acid salts which may be used in the process of the invention there may be mentioned sulphuric acid, acetic acid, formic acid, phosphoric acid and sodium dihydrogen phosphate, and as examples of the alkalis, alkaline salts, or salts which become alkaline when heated, which may be used in the process of the invention there may be mentioned sodium carbonate, sodium bicarbonate, sodium acetate, sodium hydroxide, trisodium phosphate, disodium hydrogen phosphate, sodium trichloroacetate, barium hydroxide, lithium hydroxide, sodium silicate, potassium carbonate and potassium hydroxide.

10 20 If desired mixtures of acids and/or acid salts or mixtures of alkalis and/or alkaline salts may be used in the process of the invention.

If desired the process of the invention may be carried out at a temperature above 100° C., for example at temperatures between 100° C. and 130° C. under superatmospheric pressure.

25 There may also be present in the dyebath substances which are commonly used in the dyeing of natural and regenerated protein textile materials, such as sodium sulphate or urea, or there may be present anionic surface-active agents such as the disodium salt of methylene dianthraquinone sulphonic acid, and non-ionic agents such as condensates of ethylene oxide with an amine fatty alcohol or an alkylphenol.

30 35 The dyestuffs used in the process of the invention wherein X represents



40 45 may be obtained by reacting the corresponding water-soluble dyestuff containing at least one



group with acryloyl chloride.

The dyestuffs used in the process of the invention wherein X represents  $-\text{SO}_2-$  may be obtained by treating the corresponding dyestuff containing at least one  $-\text{SO}_2\text{CH}_2\text{CH}_2\text{OH}$  group with sulphuric acid to form the sulphate ester and subsequently treating with sodium hydroxide.

50 55 Specific examples of water-soluble dyestuffs containing at least one group of the formula  $-\text{X}-\text{CH}=\text{CH}_2$ , wherein X has the meaning stated above, which may be used in the process of the invention are described in British specifications Nos. 712,037, 776,265, 787,986 and 831,128, and in Belgian specifications Nos. 565,279, 565,447, 569, 964, 573,862, 576,105 and 577,140. It is however preferred that the dyestuffs used in the process of the invention are water-soluble dyestuffs containing at least one acryloylamino group.

60 65 As examples of natural and regenerated protein textile materials which may be dyed by the process of the invention there may be mentioned textile materials com-

prising wool and silk fibres and regenerated protein fibres made from casein or ardein, and leather.

By the process of the invention there are obtained on natural and regenerated protein textile materials uniform dyeings in a wide range of bright shades which are free from the fibre to fibre unlevelness known to the trade as skitteriness and which have excellent fastness to rubbing and to wet treatments such as washing and milling.

The invention is illustrated but not limited by the following examples in which the parts and percentages are by weight:

*Example 1*

0.2 part of the dyestuff disclosed in Example 6 of British specification No. 712,037 is dissolved in 20 parts of water and the solution so obtained is added to 1000 parts of water containing 1.6 parts of a sulphuric acid and 2 parts of sodium sulphate. 20 parts of wool serge are placed in the dyebath thus obtained which is then heated to 100° C. and maintained at this temperature for 30 minutes. 6 parts of trisodium phosphate are then added and dyeing is continued for a further 45 minutes at a temperature of 100° C. The dyed wool serge is then removed from the dyebath, rinsed in water and dried.

The wool serge is dyed a uniform bright blue shade possessing much better fastness to wet treatments than wool serge which was dyed as described above except that the trisodium phosphate was not added to the dyebath.

*Example 2*

0.2 part of the sodium salt of 1-(4'-acryloylamino-phenyl)-3-methyl-4-(o-sulphophenylazo)-5-pyrazolone is dissolved in 20 parts of water and the solution so obtained is added to 1000 parts of water containing 0.6 part of sulphuric acid and 2 parts of sodium sulphate. 20 parts of wool serge are immersed in the dyebath thus obtained which is then heated to 100° C. and maintained at this temperature for 30 minutes. 1.5 parts of trisodium phosphate are then added and dyeing is continued for a further 45 minutes at a temperature of 100° C. The dyed wool serge is then removed from the dyebath, rinsed in water and dried.

The wool serge is dyed a uniform bright greenish-yellow shade possessing much better fastness to wet treatments than wool serge which was dyed as described above except that the trisodium phosphate was not added to the dyebath.

The dyestuff used in the above example may be obtained by coupling diazotised orthanilic acid with 1-(4'-acryloylaminophenyl)-3-methyl-5-pyrazolone.

*Example 3*

A solution of 0.2 part of the monosodium salt of 2-acryloylamino-7-(2'-methoxyphenylazo)-8-naphthol-6-sulphonic acid in 20 parts of water is added to 1000 parts of water containing 0.6 part of phosphoric acid and 2 parts of sodium sulphate. 20 parts of wool serge are immersed in the dyebath thus obtained which is then heated to 100° C. and maintained at this temperature for 30 minutes. An aqueous solution containing 2 parts of disodium hydrogen phosphate crystals are then added and dyeing is continued for a further 60 minutes at a temperature of 100° C. The dyed wool serge is then removed from the dyebath, rinsed in water and dried.

The wool serge is dyed a uniform bright bluish-red shade possessing much better fastness to wet treatments than wool serge which was dyed as described above except that the aqueous solution of disodium hydrogen phosphate was not added to the dyebath.

The dyestuff used in the above example may be obtained by coupling diazotised o-anisidine with 2-acryloylamino-8-naphthol-6-sulphonic acid in alkaline medium.

*Example 4*

20 parts of worsted yarn are immersed in a dyebath comprising a solution of 0.2 part of the monosodium salt

of 1-acryloylamino-8-(2'-sulphophenylazo)-7-naphthol, 1 part of sulphuric acid and 2 parts of sodium sulphate in 1000 parts of water, and the dyebath is then heated to 100° C., and maintained at this temperature for 30 minutes. 3 parts of sodium trichloroacetate are then added and dyeing is continued for a further hour at 100° C. The dyed yarn is then removed from the dyebath, rinsed in water and dried.

The worsted yarn is dyed a uniform reddish-orange shade possessing much better fastness to wet treatments than worsted yarn which was dyed as described above except that the 3 parts of sodium trichloroacetate were not added to the dyebath.

The dyestuff used in the above example may be obtained by coupling diazotised orthanilic acid with 1-acryloylamino-7-naphthol in alkaline medium.

*Example 5*

A solution of 0.5 part of the 1:2-chromium complex of 1-acryloylamino-8-(2'-hydroxy-4'-sulphamylphenylazo)-7-naphthol in 20 parts of water is added to 4000 parts of water containing 3 parts of ammonium acetate. 100 parts of wool serge are immersed in the dyebath so obtained which is then heated to 100° C. during 30 minutes. Disodium hydrogen phosphate is then added until the pH of the dyebath is 7.5 and dyeing is continued for a further 15 minutes at 100° C. The dyed wool serge is then removed from the dyebath, rinsed in water and dried.

The wool serge is dyed a uniform grey shade possessing much better fastness to a potting treatment than wool serge which was dyed as described above except that the disodium hydrogen phosphate was not added to the dyebath.

*Example 6*

20 parts of wool serge are immersed in a dyebath comprising a solution of 0.2 part of the disodium salt of 1-amino-4-[4'-acryloylamino - 3' - sulphoanilino]-anthraquinone-2-sulphonic acid, 0.6 part of sulphuric acid and 2 parts of sodium sulphate in 1000 parts of water, and dyeing is then carried out for 30 minutes at 100° C. 1.5 parts of trisodium phosphate are then added and dyeing is continued for 1½ hours at 100° C. The dyed wool serge is then removed from the dyebath, rinsed in water and dried. The wool serge is dyed a uniform bright greenish-blue shade possessing much better fastness to wet treatments than wool serge which was dyed as described above except that the trisodium phosphate was not added to the dyebath.

The dyestuff used in the above example may be obtained by treating 1-amino-4-(4'-amino-3'-sulphoanilino)-anthraquinone-2-sulphonic acid with acryloyl chloride in the presence of pyridine and converting the resulting product to the disodium salt.

*Example 7*

In place of the 0.2 part of the dyestuff used in Example 6 there is used 0.2 part of the sodium salt of 1-[β-(2' - carboxyphenylazo)acetoacetylarnino] - 4 - acryloylaminobenzene whereby the wool serge is dyed a uniform bright greenish-yellow shade.

The dyestuff used in the above example may be obtained by coupling diazotised anthranilic acid with 1-acetoacetylarnino-4-acryloylaminobenzene.

The following table gives further examples of dyeings obtained on wool serge by the method described in Example 5 above except that the 0.5 part of the dyestuff used in Example 5 is replaced by 0.5 part of the dyestuffs obtained by diazotising the amines listed in the second column of the table, coupling with the coupling components listed in the third column of the table and subsequently converting the resulting monoazo compounds to the 1:2-metal complexes by heating with a solution of the acetate of the metal listed in the fourth column of the table. The fifth column of the table indicates the shades obtained on wool.

| Example | Amine                                                                      | Coupling Component                                          | Metal    | Shade            |
|---------|----------------------------------------------------------------------------|-------------------------------------------------------------|----------|------------------|
| 8       | 4-methoxy-2-aminophenol                                                    | 1-acryloylamino-7-naphthol                                  | chromium | Greenish-grey.   |
| 9       | 4-nitro-2-aminophenol                                                      | 2-acryloylamino-6-naphthol                                  | cobalt   | Reddish-brown.   |
| 10      | 2-aminophenol-5-sulphonamide                                               | do                                                          | chromium | Reddish-grey.    |
| 11      | 4-acryloylamino-2-aminophenol                                              | $\beta$ -naphthol                                           | cobalt   | Violet.          |
| 12      | 2-aminophenol-4- $\beta$ -hydroxyethyl-sulphone.                           | 1-(4'-acryloylamino-phenyl)-3-methyl-5-pyrazolone           | chromium | Reddish-orange.  |
| 13      | Mixture of 4-nitro-2-amino-phenol and 4-acryloylamino-2-aminobenzoic acid. | 1-phenyl-3-methyl-5-pyrazolone                              | do       | Bluish-red.      |
| 14      | 4-nitro-2-aminophenol                                                      | 1-(4'-acryloylamino-phenyl)-3-methyl-5-pyrazolone           | do       | Reddish-orange.  |
| 15      | anthranilic acid                                                           | 1-(2'-methyl-5'-acryloylamino-phenyl)-3-methyl-5-pyrazolone | do       | Greenish-yellow. |
| 16      | 5-nitro-2-aminophenol                                                      | do                                                          | cobalt   | Red.             |

*Example 17*

In place of the 0.5 part of the dyestuff used in Example 5 there is used 0.5 part of the mixed 1:2-chromium complex of 1-acryloylamino-3-(2'-hydroxy-5'-nitrophenylazo)-4-naphthol and 1-(2'-hydroxynaphth-1'-ylazo)-6-nitro-2-naphthol-4-sulphonic acid whereby the wool is dyed a uniform black shade.

*Example 18*

20 parts of wool serve are immersed in a dyebath comprising a solution of 1 part of copper phthalocyanine 3-sulphon - N-(3'-acryloylamino-phenyl)amidesulphonamide sulphonic acid, 0.6 part of sulphuric acid, 0.2 part of cetyl trimethylammonium bromide and 0.4 part of a fatty alcohol/ethylene oxide condensate in 1000 parts of water, and the dyebath is then heated to 100° C. and maintained at this temperature for 30 minutes. 1.8 parts of trisodium phosphate are then added and dyeing is continued for a further hour at 100° C. The dyed wool serge is then removed from the dyebath, rinsed in water and dried.

The wool serge is dyed a uniform greenish-blue shade possessing much better fastness to wet treatments than wool serge which was dyed as described above except that the trisodium phosphate was not added to the dyebath.

The dyestuff used in the above example may be obtained by reacting copper phthalocyanine tetra-3-sulphon-chloride with m-acetyl-amino-aniline in aqueous medium in the presence of ammonia, heating with an aqueous solution of hydrochloric acid to hydrolyse the N-acetyl group, and subsequently condensing with acryloyl chloride in aqueous medium.

What we claim is:

1. Process for dyeing natural and regenerated protein textile materials with a water-soluble dyestuff of the class

15 consisting of azo, nitro, anthraquinone, and phthalocyanine, and which contain an acryloylamino group attached to a carbon atom of the dyestuff, which process comprises treating the textile material with an aqueous solution containing, as essential ingredients, said dyestuff and a member selected from the class consisting of acids and acid salts in sufficient amount so that the pH of the solution is less than 7, heating the solution while said textile material is treated therewith, thereafter adding a material selected from the class consisting of alkalis, alkaline salts, and salts which become alkaline on heating, in sufficient quantity so that the pH of the solution is raised to a level of about 4.5 to 8, and then continuing heating said solution until the dyeing is completed.

2. Process, as claimed in claim 1, wherein said pH is initially at least 2.

3. Process, as claimed in claim 1, wherein said solution is heated at each stage at a temperature within the range of about 80° C. to about 100° C., during said process.

4. Process, as claimed in claim 1, wherein said textile material is a woollen textile material.

## References Cited in the file of this patent

## UNITED STATES PATENTS

|                 |           |                     |                |
|-----------------|-----------|---------------------|----------------|
| 40              | 2,784,204 | Heyna et al. -----  | Mar. 5, 1957   |
|                 | 3,049,392 | Casty et al. -----  | Aug. 14, 1962  |
| FOREIGN PATENTS |           |                     |                |
| 45              | 712,037   | Great Britain ----- | July 14, 1954  |
|                 | 733,471   | Great Britain ----- | July 13, 1955  |
|                 | 965,902   | Germany -----       | Sept. 19, 1957 |
|                 | 565,279   | Belgium -----       | Mar. 15, 1958  |
|                 | 565,447   | Belgium -----       | Sept. 6, 1958  |
|                 | 569,964   | Belgium -----       | Jan. 31, 1959  |